

## UNITED STATES PATENT OFFICE

1,987,077

## PROCESS OF DECOLORIZING CELLULOSE NITRATE

Marvin J. Reid, Rochester, N. Y., assignor to  
 Eastman Kodak Company, Rochester, N. Y.,  
 a corporation of New York

No Drawing. Application October 4, 1932, Serial  
 No. 636,173

4 Claims. (Cl. 252—1)

This invention relates to the reclamation of film scrap and particularly to a process for reclaiming colored cellulose nitrate film base.

Many processes have been suggested in the past 5 for reclaiming film scrap and particularly cellulose nitrate film scrap from which the silver-halide emulsion has been removed but, until my invention, certain types of colored cellulose nitrate film base have defied reclamation, for the 10 reason that it has been impossible to remove the coloring without destroying the cellulose nitrate.

I have found that colored cellulose nitrate film scrap base may be reclaimed without ruining the cellulose nitrate if it is first bleached with a suitable bleaching bath, followed by treatment with an alcoholic solution of caustic alkali, after which the film base may be washed or leached with water or alcohol.

While the two principal steps of this process 20 have been separately known and used, either alone or in conjunction with some additional step, I have found that neither of these steps taken separately would, with any of the known supplementary treatments, operate to successfully 25 cover strongly colored cellulose nitrate film base for reuse.

Accordingly, it is among the objects of my invention to provide a process for reclaiming strongly colored cellulose nitrate film base or support 30 for reuse in the art. Other objects will appear to those skilled in the art upon a further perusal of this specification.

Many cellulose nitrate film negatives have the back (non-emulsion) side thereof strongly colored 35 or backed with a coloring or backing of some strong color or coating which will reduce or eliminate halation during the exposure of the film in the camera. These non-halation backings are frequently composed of a strongly dyed solution or 40 mixture of cellulose acetate, protein, albumin, or some other colloidal substance. While these so-called non-halation backings very effectively perform their purpose of eliminating halation, they are very difficult of removal from the cellulose nitrate film base when it is sought to recover the 45 base for reuse.

I have found that cellulose nitrate film base of this general character may be completely recovered and decolorized for reuse by first bleaching 50 the scrap (from which the emulsion has been removed) in a solution of a hypochlorite of an alkali metal, followed by treatment of the support in an alcoholic caustic solution. The treatment is, of course, more effective if the sheeting is first 55 cut into small pieces a fraction of an inch square,

although this is not essential. I may, for instance, bleach the foregoing cellulose nitrate base (from which the emulsion has been removed as, for instance, by soaking it in hot water) by bleaching it in a weak calcium hypochlorite solution at approximately 80–100° F. for about one and one half hours. Such a hypochlorite solution contains approximately .2% available chlorine. Before bleaching for approximately one and one half to two hours, the solution is acidified with 10 carbon dioxide until the liquor bleaches litmus rather readily. After bleaching the film scrap is removed from the bleach and washed in running water to remove bleaching liquor and insoluble salts which have been precipitated upon the 15 film support. I then immerse the so-treated nitrate film base scrap in an ethyl alcohol solution of approximately .2% sodium hydroxide (more or less) which is prepared by adding to the alcohol a 20 40% solution of alkali hydroxide. This alcoholic caustic solution is maintained at about 120° F. and the treatment continued for about five minutes. The alcoholic solution may then be drained off or the film scrap removed, after which it is 25 washed either in warm or hot water, or in two one hour leaches, with ethyl alcohol at 120° F., in order to remove all traces of solution, sodium hydroxide or decomposition products. A similar treatment using potassium hydroxide or other 30 well known caustic is likewise effective and operative in my process. Other alkali metal hypochlorites may also be used in place of the calcium hypochlorite.

Cellulose nitrate film scrap so treated will be 35 found to be quite clear and free from color or other backing materials which would contaminate the cellulose nitrate for reuse. The bleaching treatment does not allow reclaiming the cellulose nitrate even when followed by an alcohol leach, nor does the treatment with the alcoholic caustic 40 completely reclaim this type of cellulose nitrate film base, even when followed by an alcohol leach. Accordingly, the two principal steps involved in 45 my process are necessary to be operated in combination in order to effectively reclaim the strongly dyed or backed type of cellulose nitrate film base scrap.

What I claim, and desire to secure by Letters Patent in the United States is:

1. The process of removing difficultly removable dyed, colloidal, non-halation backings from cellulose nitrate sheeting which comprises subjecting the sheeting to the bleaching action of an alkali metal hypochlorite solution and then treat- 55

ing the sheeting with an alcoholic solution of caustic alkali.

2. The process of removing difficultly removable dyed, colloidal, non-halation backings from cellulose nitrate sheeting which comprises subjecting the sheeting to the bleaching action of an alkali metal hypochlorite solution containing about .2% available chlorine and then treating the sheeting with about a .2% solution of caustic alkali in alcohol.

3. The process of removing difficultly removable dyed, colloidal, non-halation backings from cellulose nitrate sheeting which comprises subjecting

the sheeting to the bleaching action of calcium hypochlorite solution and then treating the sheeting with an alcoholic solution of sodium hydroxide.

4. The process of removing difficultly removable dyed, colloidal, non-halation backings from cellulose nitrate sheeting which comprises subjecting the sheeting to the bleaching action of calcium hypochlorite solution containing about .2% available chlorine and then treating the sheeting with about a .2% solution of sodium hydroxide in alcohol.

MARVIN J. REID.